

Jan. 20, 1931.

O. M. PADDLEFORD

1,789,447

PAVEMENT

Filed May 17, 1926



Inventor:  
Oliver M. Paddleford;  
By Blakeslee & Brown,  
Attorneys.

## UNITED STATES PATENT OFFICE

OLIVER M. PADDLEFORD, OF HUNTINGTON PARK, CALIFORNIA

## PAVEMENT

Application filed May 17, 1926. Serial No. 109,510.

This invention relates to pavements and particularly to surfacing of roadways and the like. The invention has for an object the provision of a pavement which will protect 5 the foundation from cracking, breaking up, and from the deleterious effect of moisture thereon.

A further object is the provision of a pavement in which the surface is lasting and continuous rough usage thereof does not produce pits.

A further object is the provision of a surfacing which will increase the life of the sub-base. A further object is the provision 15 of a pavement wherein the different solid particles thereof are cushioned from one another and whereby such solid particles, which may be rock, are prevented from pulverizing by such rocks rubbing against one another when 20 the pavement is in actual use or holding heavy loads.

The invention has for further objects the provision of a pavement which is simple of manufacture inexpensive in construction and 25 very durable and generally superior to pavements now used.

The drawing illustrates in vertical section my improved pavement.

My pavement is directly applicable for the 30 surfacing of sub-bases, although it will be obvious that the type of pavement I am about to describe may be placed upon a suitable foundation providing this foundation is sufficiently hard and firm.

35 In the making of a pavement I use some material which will surround the different rocks or hard minerals within the same, and cushion such rocks or minerals from one another. If rocks are allowed to contact, heavy loads upon the same will grind one rock against the other, and this is particularly true of live loads, for the reason that there is a wave movement in the pavement. Al- 40 though this movement may be slight, nevertheless the effect upon the rocks is one that is deleterious, for the reason that the grinding process continues until pits are made in the pavement. Furthermore, it is necessary 45 that this cushioning material should have

non-compressible properties, and preferably be somewhat resilient in nature.

I may use in the present pavement rocks of different sizes, and I preferably provide three graded sizes of rocks. For instance, I use rocks which are hard, such as a granite type of rock, and the rocks are broken up and placed within a drum which is rotated and directs the rocks onto three different sizes of screens. The screens of the first would allow the quarter inch rocks to be collected while all other rocks under that size would pass through, and the rocks then delivered to further screens which would select the half inch rocks, and such rocks as would lie between a quarter inch and a half inch, and also all rocks that would lie between a half inch and one inch in size. Any form of rotary separator for rocks might be used and these rocks are collected in accordance with their different sizes.

The next step consists in providing the velvety material or the cushioning material that lies between the rocks to separate the same, and I may use for this purpose clay which is free from any material that would damage asphaltum. To this end the clay must be free from acids and of such a nature as to be extremely soft and fine. Clay, such as used in the making of pottery may be used, and I select the clay by applying the following test, viz: pulverized clay after being freed from any material that would damage asphaltum, 50 per cent of same must pass through a 100 mesh screen, and furthermore, it must be that quality of clay which when passed through the 100 mesh screen, 75 per cent of the same will, when washed with water, pass through a 200 mesh screen. Having selected the clay I then select a certain percentage of the different sizes of rocks. I may use various percentages of clay, rocks and asphaltum to meet varying conditions, the main principle being to provide a sufficient percentage of asphaltum to act as a binder for the rocks and clay, but I have found the following percentages adaptable for most conditions, namely, from 15 to 40 per cent clay, 5 to 15 per cent asphaltum, fine mineral aggregate being that size of rock

which would pass through a quarter inch screen and retained on a 20 mesh screen; medium mineral aggregate being that size which would pass through a half inch screen and retained on a quarter inch screen; and coarse mineral aggregate of a size that would pass through a one inch screen and be retained on a half inch screen. The percentages of the different mineral aggregates would in each instance vary from 20 to 40 per cent. The rocks are first heated and then they are mixed in the percentages named with the clay, and while the rocks are hot. The hot asphaltum is then added to the rocks and clay and the entire mass thoroughly agitated. In actual practice a machine may be provided, one side of which contains hot asphaltum and the other side of which has a bin within which are the mixed rocks and clay which have been heated, and between the bin for the rocks and the clay and the container for the hot asphaltum are paddles which are rotated to thoroughly mix the asphaltum and the rocks and clay. The mixed asphaltum, rocks and clay are then delivered into a suitable receptacle whereby the same may be spread upon the road foundation. The entire mix is rolled while hot.

Referring to the drawing I have shown a foundation or sub-base at 1 and the surfacing constituting the invention at 2, and the different grades of rocks, namely, the quarter inch, half inch and one inch with intervening sizes, are shown at 3. These rocks are separated by the cushion material 4 in combination with asphaltum. Rolling the mix while it is hot tends to press the rocks away from the surface and present a thin layer of asphaltum for the immediate top surface as shown at 5.

Acids have a bad effect upon asphalt, in that acids tend to eat the asphaltum and render the pavement structure weak, with the result that the rocks are allowed to contact and abrade one another, and pits and cracks occur in the pavement. As I have previously stated, the pavement material that I have described is intended primarily for use as a pavement surfacing. However, it may be used as a sub-base providing the foundation is sufficiently firm and hard. If the surfacing is placed upon concrete, it will be obvious that the concrete will be protected.

Concrete being very hard tends to rut easily if a heavy load is impacted suddenly thereon. My surfacing, however, gives a cushioning effect, and thus the blow is prevented from damaging the concrete there beneath.

Sand cannot be used in the present invention, because sand compacts, and furthermore, for the reason that sand is simply small rocks. My concept and invention requires the use of a material between the rocks which will not stay compressed, and

while I have described clay as one of such materials, yet it is obvious that other materials of like nature and with like properties might be used.

Having thus disclosed my invention, I claim and desire to secure by Letters Patent:

1. The method of constructing a roadway which consists in first preparing a paving material by heating rocks and clay and separately heating asphaltum, then mixing the hot asphaltum with the hot clay and rocks whereby the clay and asphaltum combine to produce an elastic adhesive mixture separately encasing each rock, then pouring the mass while hot upon the roadway and then rolling the mass while it is hot.

2. The method of preparing a paving material which consists in heating rocks and clay and separately heating asphaltum, then mixing the hot asphaltum with the hot clay and rocks whereby the clay and asphaltum combine to produce an elastic adhesive mixture separately encasing each rock.

In testimony whereof, I have signed my name to this specification.

OLIVER M. PADDLEFORD.

95

100

105

110

115

120

125

130